

Patented Jan. 10, 1928.

1,655,414

# UNITED STATES PATENT OFFICE.

HENRY FLORY, OF HAWTHORN, NEW JERSEY.

## METHOD AND CHEMICAL MIXTURE FOR PRODUCING BROCADED TEXTILES.

No Drawing.

Application filed October 9, 1925. Serial No. 61,519½.

The present invention relates to method, apparatus, and treating mixtures for producing brocaded fabrics. The invention relates particularly to the producing of a brocade from a fabric having a cotton back and a wool face, such as a corduroy, velvet, or plush, but is applicable to fabrics of other combinations of backing and facing. The invention further relates to the producing of a brocade and the dyeing of the different parts of the brocade in side by side, intermingled, or simultaneous steps of one process. The invention further particularly relates to the production of a brocade from a pile textile in which the pile and backing are of different materials, such for example as wool and cotton respectively, by using a chemical which will attack the wool but not the cotton, the mixture being applied to the pile over designed areas.

According to my invention a brocade of velvet, plush or other textile having pile fibres, is made by removing designed areas of the pile thereof by means of a chemical which will destroy the integrity of the fibres of the pile at the designed areas. This destruction of the pile fibre may involve the solution of the fibre or the disintegration thereof or both. The fibre destroying or "burning" mixture may be applied by printing it on by means of intaglio plate or rolls. The mixture may then be permitted to have time to attack the fibres of the pile to which it was applied and the destruction of these fibres may be hastened by the application of heat or moisture or both.

During the process of removing designed areas of the pile to produce a brocade from a suitable textile dye may be applied to the textile either to a portion or all of that part of the backing from which the pile is removed or to the pile which is left or to both in one or more colors. Color or dye may be applied to the backing by mixing it with and applying it to the textile with the burning mixture. The colors may be printed on the cloth in a textile printing machine of the sort well known in the art and means may be provided for applying the burning mixture thereby.

Other objects of my invention will appear from the specification and the claims.

According to this invention, in making a brocade from a velour having a cotton backing and a wool pile, a chemical mixture for destroying a part of the pile is made up of

the following ingredients and quantities: about 60 parts of 15% caustic soda solution by volume, one part of 15% sulphuric acid, and 140 parts 10% gum arabic solution or other strength commonly used for printing on textiles.

The mixture is applied to designed areas of the textile by printing it on the pile face with intaglio plates or, preferably, by means of a printing machine such as is commonly used on textiles. The textile is run from the printing machine to and through a steaming chamber where it is exposed to the heat and moisture of the steam for about thirty minutes, whereby the pile fibres of the areas printed are disintegrated and destroyed.

After the steaming the cloth is dried at about 200° F.

After drying the disintegrated fibres these are brushed from the cloth, after which it is washed and dried and when necessary again brushed to bring up the fibres of the pile.

After this treatment the velour, or any other like textile, has all the pile fibres in the unprinted areas in as good condition as before and the line between the unprinted areas of the pile and the backing which now shows is sharp and clear. The "burning" mixture does not spread from the printed areas and sharp pointed designs and finely lined designs may be made. The cotton of the backing is strengthened by the process and is tightened about the fibres of the pile areas not printed. The pile fibres printed are removed even entirely through the weave of the back.

Dyes may be applied at the time of printing which after the process is completed will serve as decoration for the reverse side of the textile in which case hangings, tapestries, and the like may be made which will not require lining.

Although I have shown and described and have pointed out in the annexed claims certain novel features of the invention, it will be understood that various omissions, substitutions and changes in the several steps of the process and in its operation may be made by those skilled in the art without departing from the spirit of the invention.

I claim:

1. The method of making a brocade from a textile having a cotton back and a pile face of wool which comprises impregnating designed portions of the pile face with a mixture comprising a carrier and 60 parts

by volume of 15% solution of caustic soda to one part of a 15% water solution of sulphuric acid, permitting the mixture to disintegrate the impregnated portions of the pile, and then removing disintegrated pile fibers and any remaining impregnating mixture.

2. The method of making a brocade from a textile having a cotton back and a pile face of wool which comprises impregnating designed portions of the pile face with a mixture comprising a carrier of gum arabic and 60 parts by volume of 15% solution of caustic soda to one part of a 15% water solution of sulphuric acid, permitting the mixture to disintegrate the impregnated portions of the pile, and then removing disintegrated pile fibers and any remaining impregnating mixture.

3. The method of making a brocade from a textile having a cotton back and a pile face of wool which comprises impregnating designed portions of the pile face with a mixture comprising textile printing gum arabic solution 140 parts by volume to 69 parts of 15% solution of caustic soda and one part of a 15% water solution of sulphuric acid, permitting the mixture to disintegrate the impregnated portions of the

pile, and then removing disintegrated pile fibers and any remaining impregnating mixture.

4. The method of producing a brocade from a plush, velour, or the like textile having a cotton back and a wool face which comprises printing on designed portions of the pile face with a mixture comprising textile printing gum arabic solution 140 parts by volume to 60 parts 15% solution of caustic soda solution and one part of a 15% water solution of sulphuric acid, steaming the mixture printed textile for about thirty minutes, drying at between 175° F. and 225° F., brushing the disintegrated pile fibers, and then washing and drying the textile.

5. The method of producing a brocaded fabric from a plush, velour, or the like textile having a vegetable fibre back and an animal fibre pile which comprises impregnating designed portions with a water solution of caustic soda and sulphuric acid, the concentration by weight of the caustic soda being in the neighborhood of fifty times the weight of the sulphuric acid.

In testimony whereof I have hereunto set my hand.

HENRY FLORY.